

April 14, 1970

N. H. KATZ ET AL

3,506,235

FUEL CASTING APPARATUS WITH COLLAPSIBLE CORE

Filed Sept. 12, 1967

2 Sheets-Sheet 1



INVENTORS  
NORMAN H. KATZ  
ROGER N. BEAM

BY

*Ronald A. Goodman*

ATTORNEY

April 14, 1970

N. H. KATZ ET AL

3,506,235

FUEL CASTING APPARATUS WITH COLLAPSIBLE CORE

Filed Sept. 12, 1967

2 Sheets-Sheet 2



INVENTORS  
NORMAN H. KATZ  
ROGER N. BEAM

BY

*Norman H. Katz*

ATTORNEY

## 1

3,506,235

### FUEL CASTING APPARATUS WITH COLLAPSIBLE CORE

Norman H. Katz, Northridge, and Roger N. Beam, Chatsworth, Calif., assignors, by mesne assignments, to the United States of America as represented by the United States Atomic Energy Commission

Filed Sept. 12, 1967, Ser. No. 667,638

Int. Cl. B29c 11/00

U.S. Cl. 249—82

3 Claims 10

#### ABSTRACT OF THE DISCLOSURE

Apparatus disclosure and method for casting an annular uranium carbide and other nuclear fuel elements. The mold includes a solid graphite rod within an annular graphite core. The core is designed to collapse upon cooling of the molded fuel, while the graphite rod serves as a heat sink for the mold to prevent premature destruction of the core. The core and rod in one embodiment are separated by an air gap clearance sufficient to permit the molded fuel to contract when cooling without destroying the hollow core. In another embodiment, the solid rod is sectioned and includes graphite spacer rings for permitting expansion and contraction of the rod sections to thereby provide intimate thermal contact between core and rod when the fuel is molten, while permitting contraction of the rod segments as the fuel cools.

#### BACKGROUND OF THE INVENTION

The invention relates to casting annular shaped fissile fuel such as uranium carbide or oxide. More particularly, the invention relates to a particular method and apparatus for such casting. This invention arose in the course of, or under, Contract AT(38-1)-430 with the United States Atomic Energy Commission.

Uranium carbide is a well known fuel element for nuclear reactors. One method for producing such fuel elements is by casting. Normally, such fuel elements are in the form of rods so that casting presents no particular difficulty.

The casting of annular fuel elements has been difficult because of high coefficient of thermal expansion and the inherent brittleness of uranium carbide. These characteristics limit both the amount of machining which may be performed on such cast elements and limit the obtaining of any controlled dimensions for the casting.

When such elements have been cast using solid graphite cores, substantial cracks frequently develop in the uranium carbide during the cooling process because of the differential expansion between the cast UC and solid graphite core.

#### SUMMARY OF THE INVENTION

Accordingly, it is an object of this invention to provide substantially crack-free cast UC.

Another object is to provide cast UC having controllable dimensions.

A further object is to provide improved annular fissile fuel elements.

The invention provides these and other objects by using

## 2

a molding process including an annular graphite core enclosing a solid core both within a mold casing, the annular core being designed to collapse when the molded metal cools and the solid core serving as a heat sink during the cooling process. Two embodiments are disclosed, one having an air gap between the solid and annular core, while the other embodiment has a collapsible solid core.

#### DESCRIPTION OF THE DRAWING

FIGURE 1 illustrates one embodiment of the invention in an exploded view.

FIGURE 2 illustrates a second embodiment of the invention in an exploded view.

FIGURE 3 illustrates one form of a multiple mold casting apparatus.

FIGURE 4 illustrates a third embodiment of the invention in an exploded view.

#### DESCRIPTION OF THE INVENTION

FIGURE 1 illustrates one form of the invention for making annular fuel element  $\frac{3}{4}$ " in diameter by  $\frac{1}{4}$ " thick and approximately 3" high.

An annular mold body or casing 1 may be of graphite or metal. The casing is closed at the bottom by a plug 2 having a circular recess 3.

The top of the casing is open and has a ridge 9 for supporting the plug 4. The top plug 4 also includes a centrally located circular recess 5. The top and bottom plugs serve as support and centering plates for the annular hollow graphite core 6 and the solid graphite heat sink 7 which fit within the recesses 3 and 5 as shown.

The top plug 4 also serves as a distributor of the liquid uranium carbide which is poured into the body of the mold casing to form the annular casting. The plug 4 is essentially a disc having four arms or salient poles 8 which extend therefrom and are supported on the ridge 9 of casing 1.

In the process of casting, molten uranium carbide is prepared in an argon atmosphere at 23 inches of mercury pressure, and is poured at 2500° C.

The molten metal is poured onto and distributed by the distributor cap 10 of the top plug 4; it flows in the voids between the arms 9 into the  $\frac{1}{4}$ " annular space 11 formed in the mold.

The thin wall elongated hollow graphite core 6 in all embodiments of the invention is designed sufficiently strong to restrain molten UC, but low enough so that it will crack due to the contraction existing in the UC when cooled. In FIGURE 1, this tube is .010 inch thick and has a  $\frac{1}{4}$  inch diameter.

An air gap 12 exists between the hollow core 6 and solid graphite core 7. The air gap is quite small since the solid core 7 serves primarily as a heat sink to distribute the liquid metal heat by conduction to the casing members 1, 2 and 4. The air gap space ideally is equal to the contraction experienced by the fuel in cooling.

FIGURE 2 illustrates a second embodiment of the invention designed for casting 2" diameter cores having the same  $\frac{1}{4}$ " thickness as in FIGURE 1. Essentially, FIGURE 2 is very similar to FIGURE 1 with several exceptions. The same numerals are used as in FIGURE 1 for corresponding parts. The air gap 12 between hollow core 6 and solid core 7 is larger—of the order of .042 inch.

Because of the larger size of all the elements, the method of alignment and centering of the solid core 7 is slightly different. The heat sink action of FIGURE 2 must be more efficient than in FIGURE 1. Accordingly, the solid core 7 has a cap or extension 13 adapted for mating with the opening 14 in distributor plate 4. Thus the extension can radiate heat directly to the atmosphere as well as conductively through the distributor. The bottom plate 2 includes a ridge 15 for supporting hollow core 6 and spacing it from the solid core 7 which is supported on the bottom of the plate.

FIGURE 3 illustrates a multiple mold casting method utilizing five molds of the type in FIGURES 1, 2 and 4. One of the problems encountered with multiple molding is that the temperature of the liquid metal is usually higher and there is a greater possibility of destroying the hollow core during casting.

Accordingly, a large conical graphite distributor 16 is used to provide a laminar flow into the mold cavities. Liquid metal is poured from a ladle or other means onto this distributor. A tube 17 is shown to illustrate the direction of pouring. This distributor device has proven quite effective in providing just sufficient chilling of the molten UC to protect the cores. The use of a flat distributor caused too much chilling and resulted in unacceptable mold.

FIGURE 4 illustrates a third embodiment of the invention which is particularly suitable for large castings and other applications where more heat is generated than can be dissipated by the embodiments shown in FIGURES 1 and 2. This embodiment resembles those previously discussed in that it includes a mold cavity 11 defined by cylindrical outer casing or body 1, hollow collapsible core 6, and base plate 2; a top plate or distributor 4; and an inner core or heat sink 7. It differs from FIGURES 1 and 2 in that there is no air gap between hollow core 6 and heat sink core 7, the two cores being in direct contact with each other, thereby providing more effective transfer of heat from the casting.

Heat sink core 7 comprises an assembly of three or more elongated pie-shaped segments 27 linked together by resilient members or springs 20 and shown separated by air gaps 28 in the normal or hot conditions. For purposes of illustration, four segments 27 are shown in FIGURE 4. Graphite spacer springs 20 tend to expand core assembly 7 radially, such that each of its segments 27 is pressed in direct contact against the inner surface of hollow core 6. At the same time, springs 20 are flexible enough to permit core assembly 7 to collapse along with hollow core 6 as the casting cools and contracts, thereby closing the air gaps. In the drawing, springs 20 are shown as resilient C-rings operating in slots in the top and bottom of core segments 27.

The spring-loaded core assembly 7 in this embodiment tends to center itself within core 6. Hence, additional centering means such as the peg and hole arrangement, 13 and 14, in FIGURE 2 is unnecessary. In FIGURE 4, the opening 14 in top plate 2 is closed with plug 24.

Subsequently, as the liquid metal cools in annular space 11 and the annular fuel element contracts, the spacer rings 20 are compressed and contract until limited by the meeting of the four segments in the center of the mold with the elimination of air gaps 28.

The advantage of the apparatus of FIGURE 4 is that the solid core is always in direct thermal contact with the hollow core and the liquid metal, while yet permitting contraction of the fuel element. Thus this embodiment is especially adapted for large fuel element casting.

The embodiment depicted in FIGURE 4 has produced crack-free uranium carbide fuel elements as large as 6 inches long and 3½ inches in diameter, with a ¼-inch wall thickness, thus illustrating the merit of combining a flexible core with efficient heat transfer means.

While the invention has been described as required,

the chart below indicates the relevant factors in design for several sizes of molds:

TABLE 1.—DIMENSIONS OF SINGLE-CAVITY GRAPHITE MOLDS AND AS-CAST CYLINDERS

| Mold dimensions (in.) | Casting dimensions                                          |                                         | Shrinkage ( $\Delta D$ ) (in.)    |
|-----------------------|-------------------------------------------------------------|-----------------------------------------|-----------------------------------|
|                       | Nominal                                                     | OD by ¼ in. ID by 3 in. long UC casting |                                   |
| 10                    | Outer mold tube: OD, 1,000<br>ID, 0.750                     | OD: Top, 0.724<br>Bottom, 0.720         | OD: Top, -0.026<br>Bottom, -0.030 |
|                       | Inner shell core OD, 0.270                                  | ID: Top, 0.267                          | ID: Top, -0.003                   |
|                       | Solid core insert OD, 0.240                                 | Bottom, 0.266                           | Bottom, -0.004                    |
| 15                    | Nominal 2,000 in. OD by 1.5 in. ID by 3 in. long UC casting |                                         |                                   |
|                       | Outer mold tube: OD, 2,375<br>ID, 2,000                     | OD: Top, 1.937<br>Bottom, 1.935         | OD: Top, -0.063<br>Bottom, -0.065 |
|                       | Inner shell core: OD, 1,520<br>ID, 1,500                    | ID: Top, 1.490<br>Bottom, 1.488         | ID: Top, -0.030<br>Bottom, -0.032 |
| 20                    | Solid core insert OD, 1,430                                 |                                         |                                   |
|                       | Nominal 3,500 in. OD by 3 in. ID by 1½ in. long UC casting  |                                         |                                   |
|                       | Outer mold tube: OD, 4,000<br>ID, 3,500                     | OD: Top, 3,395<br>Bottom, 3,390         | OD: Top, -0.105<br>Bottom, -0.110 |
| 25                    | Inner shell core: OD, 3,000<br>ID, 2,970                    | ID: Top, 2,930<br>Bottom, 2,930         | ID: Top, -0.070<br>Bottom, -0.070 |
|                       | Solid core insert OD, 2,855                                 |                                         |                                   |

TABLE 2.—DIAMETRICAL SHRINKAGE OF CAST ANNULAR UC FUEL

| Nominal<br>as-cast<br>cylinder OD<br>(in.) | Diametrical shrinkage (in.) |       |            |       |
|--------------------------------------------|-----------------------------|-------|------------|-------|
|                                            | Measured (avg.)             |       | Calculated |       |
|                                            | OD                          | ID    | OD         | ID    |
| 35                                         | 0.028                       | 0.004 | 0.022      | 0.007 |
| 2,000                                      | 0.064                       | 0.031 | 0.060      | 0.045 |
| 3,500                                      | 0.107                       | 0.070 | 0.104      | 0.089 |

While several embodiments of the invention have been described, it will be obvious that modification can be made thereto. Furthermore, the invention has been described with reference to uranium carbide and other brittle nuclear fuel elements. However, it is anticipated that the invention may find use in other and less critical casting applications. Accordingly, the invention is defined in the following claims.

What is claimed is:

1. Apparatus for casting annular elongated fuel elements comprising: an elongated hollow casing having an open end and a closed end; a thin, elongated annular hollow graphite core and a second graphite core within and coextensive with said hollow core; and a graphite distribution plate having a plurality of salient poles positioned for substantially closing the open end of said casing and for positioning both cores with their axes coaxial with said casing, whereby a cavity is formed between the inside diameter of the casing and the outer diameter of the hollow core, said second core including a plurality of elongated coextensive spaced segments of solid graphite and a resilient graphite ring-type spring adapted for permitting expansion and compression of said segments in unison in intimate contact with the inner circumference of the hollow core while the poured liquid metal cools.
2. Apparatus for casting annular elongated fuel elements comprising: an elongated hollow casing having an open end and a closed end; a thin, elongated annular hollow graphite core and a second graphite core within and coextensive with said hollow core; and a graphite distribution plate having a plurality of salient poles positioned for substantially closing the open end of said casing and for positioning both cores with their axes coaxial with said casing, whereby a cavity is formed between the inside diameter of the casing and the outer diameter of the hollow core, said second core including a plurality of elongated coextensive spaced segments of solid graphite

and a resilient graphite ring-type spring adapted for permitting expansion and compression of said segments in unison in intimate contact with the inner circumference of the hollow core while the poured liquid metal cools, said segments being spaced from each other a distance corresponding to the contraction of liquid metal in the cavity when cooled.

3. Apparatus for casting elongated annular fuel elements, comprising:

- (a) an elongated hollow casing having an open end 10 and a closed end;
- (b) a thin, elongated hollow core positioned within said casing such that an elongated annular mold cavity is formed having one open end and one closed end between the casing and the hollow core; 15
- (c) a flexible heat sink core assembly within the hollow core, comprising a plurality of elongated pie-shaped segments linked together by resilient means, for maintaining the core segments in intimate contact with the inner surface of the hollow core, and 20 for permitting the assembly to contract with the

hollow core as metal poured into the mold cavity cools; and

(d) a distributor plate located at the open end of the casing and cavity for centering the cores within the casing and for sealing off the volume within the hollow core from the flow of metal poured into the mold cavity.

#### References Cited

#### UNITED STATES PATENTS

|           |         |             |       |           |
|-----------|---------|-------------|-------|-----------|
| 773,590   | 11/1904 | Rafter      | ----- | 249—107   |
| 1,946,451 | 2/1934  | Bailey      | ----- | 249—175 X |
| 2,779,676 | 1/1957  | Brownstein. |       |           |
| 2,405,254 | 8/1946  | Hopkins     | ----- | 249—82 X  |
| 2,583,248 | 1/1952  | Bajrovic    | ----- | 249—82 X  |

ROBERT D. BALDWIN, Primary Examiner

U.S. Cl. X.R.

249—107, 122, 134, 177